

[54] STEEL BAR STOCK AND METHOD FOR  
MAKING SAME

[76] Inventor: Hugh M. Gallagher, Jr., 7262 State Rd., Cincinnati, Ohio 45230

[22] Filed: Dec. 29, 1972

[21] Appl. No.: 319,499

[52] U.S. Cl..... 148/12 B; 148/12 B

[51] Int. Cl..... C21d 7/02

[58] Field of Search..... 148/12 B, 36; 75/123 N,  
75/123 J

## [56] References Cited

## UNITED STATES PATENTS

|           |        |               |          |
|-----------|--------|---------------|----------|
| 2,933,424 | 4/1960 | Canney et al. | 148/12 B |
| 3,230,118 | 1/1966 | Tufts         | 148/12 B |
| 3,668,020 | 6/1972 | Lucht         | 148/12 B |

Primary Examiner—W. Stallard  
Attorney, Agent, or Firm—Melville, Strasser, Foster & Hoffman

## [57] ABSTRACT

A high strength fine grain killed steel consisting essentially of, by weight percent:

|            |              |
|------------|--------------|
| carbon     | 0.50 – 0.55% |
| manganese  | 1.20 – 1.65% |
| phosphorus | 0.040% max.  |
| sulfur     | 0.050% max.  |
| silicon    | 0.30% max.   |
| vanadium   | 0.03 – 0.05% |
| iron       | Balance,     |

and processed into bar stock by the steps which include, hot reducing to substantially final gauge, rapidly cooling the hot reduced stock, cold finishing up to about 15%, and stress relieving between about 500° and 850° F. Said steel has particular utility for threaded bolts, such as "U" bolts, as the ductility is relatively high, permitting thread rolling and forming without additional heat treatment and cleaning.

6 Claims, No Drawings

## STEEL BAR STOCK AND METHOD FOR MAKING SAME

### BACKGROUND OF THE INVENTION

The present invention relates to a high strength steel in bar stock form, and more particularly to the use of said steel in threaded fasteners, such as "U" bolts.

This development arose from a need in the automotive industry for a relatively low cost, high strength steel having a sufficiently high ductility to permit thread rolling and forming into a "U" shape. Such members, in nominal sizes ranging from  $\frac{1}{4}$  to  $1\frac{1}{2}$  inches, are used in fastening the springs to the axles of trucks and automobiles. Since high strength and good fatigue properties are obvious prerequisites for such threaded fasteners, it was necessary for the automotive industry to turn to the alloy steels such as AISI Type 4140. However, the material and processing costs for said steels are quite high, particularly when compared with such costs for the steels of this invention.

In any case, the minimum mechanical and quality requirements for externally threaded fasteners under SAE J429d, for Grade 8 screws and studs in sizes between  $\frac{1}{4}$  and  $1\frac{1}{2}$  inches, are as follows:

|                        |          |
|------------------------|----------|
| Tensile Strength (psi) | 150,000  |
| Yield Strength (psi)   | 130,000  |
| Elongation in 2" (%)   | 12       |
| Reduction in Area (%)  | 35       |
| Hardness (Rc)          | 32 - 38. |

As noted above, it was necessary to use alloy steels, such as AISI Type 4140 (Quenched and Tempered) to achieve these minimum requirements. The use of this material meant following a processing sequence not suited for developing maximum economy. For example, due to the undesirability of cut threads, which practice can materially affect the fatigue properties of the bar stock, a roll threading step had to be followed. As a consequence, said operation had to be conducted prior to the quench and temper, which necessitated a cleaning and often straightening before use could be made of the bolt.

The present invention avoids these inherent problems by a combination of chemistry and processing controls.

### SUMMARY OF THE INVENTION

The present invention contemplates a simplified processing sequence to produce a high strength, fine grained, killed steel bar stock, more particularly bar stock for use as threaded fasteners.

The steel of this invention is basically a medium high carbon steel, and consists essentially of about, by weight percent, the following:

|            |          |      |       |
|------------|----------|------|-------|
| carbon     | 0.50     | -    | 0.55% |
| manganese  | 1.20     | -10  | 1.65% |
| phosphorus | 0.040%   | max. |       |
| sulfur     | 0.050%   | max. |       |
| silicon    | 0.30%    | max. |       |
| vanadium   | 0.03     | -    | 0.05% |
| iron       | Balance. |      |       |

However, chemistry alone is not the answer, as a controlled processing sequence must be followed.

Briefly, in the practice of this invention, a steel having the foregoing chemistry is subjected to various metallurgical operations which include, hot rolling the steel

into bar stock to within 10% to 15% of final gauge without coiling, severing the stock into individual pieces to allow for the rapid cooling thereof, cold finishing to final bar size, and stress relieving at a temperature between about 500° and about 850° F. The stock may now be roll threaded, formed and shipped without the necessity of cleaning and straightening distorted parts. When tested, it will be found to possess substantially the mechanical and quality requirements of Grade 8 material, under SAE J429d.

### DETAILED DESCRIPTION OF THE PREFERRED EMBODIMENT

This invention relates to a killed steel consisting essentially of, by weight percent:

|            |          |      |       |
|------------|----------|------|-------|
| carbon     | 0.50     | -    | 0.55% |
| manganese  | 1.20     | -    | 1.65% |
| phosphorus | 0.040%   | max. |       |
| sulfur     | 0.050%   | max. |       |
| silicon    | 0.15     | -    | 0.30% |
| vanadium   | 0.03     | -    | 0.05% |
| iron       | Balance, |      |       |

which when processed into bar stock in the manner to be described hereinafter, will have a fine grained structure between about A.S.T.M. No. 5-8, and meet the following minimum properties:

|                        |   |          |
|------------------------|---|----------|
| Tensile Strength (psi) | - | 150,000  |
| Yield Strength (psi)   | - | 130,000  |
| Elongation in 2" (%)   | - | 12       |
| Reduction in area (%)  | - | 35       |
| Hardness (Rc)          | - | 32 - 38. |

Before discussing the processing sequence in detail, it should be noted that the preceding minimum properties are those required for Grade 8 material under SAE Standard J429d. This SAE Standard covers the mechanical and quality requirements for steel bolts, screws, studs, and sems used in automotive and related industries in sizes to  $1\frac{1}{2}$  inches, inclusive.

In today's age, where high speed personal transportation is quite common, one clear and essential requirement is that the transportation means, such as truck, automobile, bus, etc., be as safe as practical considerations will allow. But along with this, such means must be economical, or the vehicle would remain nothing more than a drawing board concept. The present invention recognizes this, for it relates to a cost cutting material suitable for use in assembling the vehicles, without jeopardizing the safe performance thereof.

Turning now to the processing sequence, in the practice of this invention, a steel, preferably having a chemistry falling within the ranges above, and preferably one having a minimum of 1.50% by weight Mn, is subjected to a standard hot reducing operation to within 10% to 15% of final gauge. However, instead of coiling the hot reduced bar stock, following said hot reduction, the stock is cut or severed into individual lengths for rapid air cooling. This is in contrast to the slow cooling of a wound coil of hot steel. It was discovered with said high carbon steels, that with rapid cooling, the formation of pearlite could be avoided. However, as cooling rates decreased, the tendency for pearlite formation increased.

The individual lengths of hot reduced bar stock are then subjected to a cold finishing to final gauge.

It was then discovered that contrary to what would be expected, a significant increase in properties could be realized with a controlled stress relieving step. Specifically, it was found that the yield strength could be increased by as much as 20,000 psi with a stress relief between about 500° F. and about 850° F., for about 1 hr. This may be demonstrated by the comparison which follows.

### EXAMPLES

A heat of steel, whose chemistry is as follows, by weight percent:

|            |          |
|------------|----------|
| carbon     | 0.51%    |
| manganese  | 1.57%    |
| phosphorus | 0.013%   |
| sulfur     | 0.033%   |
| silicon    | 0.30 %   |
| vanadium   | 0.043%   |
| iron       | Balance. |

is processed in the preferred manner above into .680 in. rounds, and subsequently stress relieved over a range of temperatures. The results, as expressed in mechanical properties, are listed below:

TABLE

| Treatment       | Tensile Strength<br>(psi) | Yield Strength<br>(psi) | Elongation<br>in 2" (%) |
|-----------------|---------------------------|-------------------------|-------------------------|
| drawn           | 158,000                   | 111,000                 | 15                      |
| stress Relief   |                           |                         |                         |
| nealed: 400° F. | 160,000                   | 115,000                 | 13                      |
| stress Relief   |                           |                         |                         |
| nealed: 500° F. | 166,500                   | 135,000                 | 12                      |
| stress Relief   |                           |                         |                         |
| nealed: 600° F. | 167,000                   | 137,000                 | 14.5                    |
| stress Relief   |                           |                         |                         |
| nealed: 800° F. | 162,500                   | 133,000                 | 15                      |

NOTE: values are averages from up to four samples - grain sizes between about A.S.T.M. No. 5

The preceding data clearly shows the significance of the critical stress relief given the steels of this invention. However, it should be emphasized that said results are due in part to the chemistry of the steel. For example, several companion heats, having no vanadium and containing lesser amounts of manganese, were treated along with the last samples above, and found to be relatively low in mechanical properties. Specifically, the latter could not meet the SAE standard noted above. Since modifications may be made in the processing of the steels of this invention, particularly by the skilled worker after reading these specifications, no limitation is intended to be imposed herein except as set forth in the appended claims.

The embodiments of the invention in which an exclusive property or privilege is claimed are defined as follows:

1. A method of making ferrous bar stock in sizes up about 1½ inches diameter, comprising the steps of

hot reducing to within 10% to 15% of final gauge in straight lengths, a killed ferrous alloy consisting essentially of carbon between about 0.50 - 0.55% by weight, manganese between about 1.20 - 1.65% by weight, vanadium between about 0.03 - 0.05% by weight, with the balance substantially all iron, cold finishing said hot reduced stock to final gauge, and stress relieving said stock at a temperature between about 500° F. - 850° F.

2. The method according to claim 1 including the step of roll threading the stress relieved bar stock to form threaded fasteners.

3. The method according to claim 1 wherein said hot reduced bar stock is rapidly cooled to avoid any substantial formation of pearlite.

4. The method according to claim 3 wherein said hot reduction is conducted as a continuous step, whereas the cold finishing is conducted on cut lengths of said hot reduced bar stock.

5. The method of making an automotive U-bolt in sizes up to about 1½ inches diameter, comprising the steps of hot reducing to within 10% to 15% of final gauge, in straight lengths, a medium high carbon steel,

cold finishing said hot reduced stock to final gauge, stress relieving said stock at a temperature between about 500° F. and 850° F., cutting said stock to length, thread rolling, and then cold forming said cut and threaded lengths into U-shape.

6. The method of making an automotive U-bolt in sizes up to about 1½ inches diameter, comprising the steps of hot reducing to within 10% to 15% of final gauge, in straight lengths, a killed ferrous alloy consisting essentially of carbon between about 0.50% and 0.55% by weight, manganese between about 1.20% and 1.65% by weight, vanadium between about 0.03% and 0.05% by weight, with the balance substantially all iron, cold finishing said hot reduced stock to final gauge,

stress relieving said stock at a temperature between about 500° F. and 850° F., cutting said stock to length, thread rolling, and then cold forming said cut and threaded lengths into U-shape.

\* \* \* \* \*